

## UNITED STATES PATENT OFFICE

2,036,848

METAL CLEANSING COMPOSITION AND  
METHOD

Frank Amthor, East Rutherford, and George C. Reinhard, Wood-Ridge, N. J., assignors to American Colloid Corporation, New York, N. Y., a corporation of New York

No Drawing. Application September 9, 1933,  
Serial No. 688,824

11 Claims. (Cl. 87—5)

This invention relates to improvements in methods for the cleansing of metals and metal parts which have become fouled by the accumulation thereon of oil and grease and more particularly for the cleansing of such metal parts as the cooling circulating systems of internal combustion engines, as automobile radiators, and the like, which, on account of their construction are not readily accessible so that it is desirable to accomplish the cleansing thereof, without the aid of any mechanical device whatsoever except such incidental mechanical aid as may be derived from the circulation of the cleansing solution itself.

15 Metal parts such as automobile radiator cores and the like become fouled by the accumulation on the surface thereof, of dirt, rust, oil and grease. On account of their construction, such parts are not readily accessible so that a practical chemical means for cleansing is desired. Examination shows that the solid particles as dirt and rust are attached to the surface by means of a film of oil or grease in a highly emulsified state with water and in order to remove such 25 foreign material, it is essential to remove the layer of emulsified grease or oil.

Where organic solvents are used for the cleansing of such metal parts as the interiors of automobile radiators, practical difficulties arise from 30 the standpoint of cost and manipulation and the results are not entirely efficacious. The oil or grease attached to the metal surfaces under consideration being emulsified with water, wetting out by anhydrous water repellent organic 35 grease solvents is not entirely practical, so that the grease removal would be incomplete; moreover, after application of such organic grease solvents, they would be flushed by means of water, a non-miscible medium, with the tendency to 40 leave a deposit of a film on which additional dirt would accumulate most readily. Where oil emulsions or emulsifying agents alone are used, the bond between the greasing accumulation and the metal walls is not sufficiently weakened to 45 render such agencies practical.

It is among the objects of the invention to provide compositions of matter, easily prepared from inexpensive ingredients, which do not lose 50 their efficacy, though used long after preparation thereof, which may be easily introduced into the cooling circulating systems of internal combustion engines for quickly and effectively removing the accumulation of oil, grease, dirt or rust from 55 metal parts that are subjected to water contact,

which composition will not boil at low temperatures and will involve no fire hazard.

It is among other objects of the invention to provide a method for cleansing metal parts, such as those of cooling circulating systems of internal combustion engines that have become 5 fouled by the accumulation of oil, grease, dirt or rust, by which method a relatively effective reaction is caused to take place as the cleansing composition reaches the accumulation for effective removal of the latter. 10

Broadly we accomplish the desired result by effecting and permitting a combination directly at the parts to be cleansed, of two distinct complementary ingredients of an emulsifying agent, 15 all in the presence of an organic solvent.

The invention is preferably carried out by the use of a fatty acid, as one of the ingredients of the emulsifying agent, which would be saponified directly at the parts to be cleansed, by the reaction 20 with the complementary or alkaline ingredient.

In a preferred application, according to our invention, the two distinct ingredients of the emulsifying agent, are applied successively. In 25 the first stage, the accumulation to be removed is conditioned, for effective action thereon of the reaction composition applied in the second stage. As the conditioning composition we preferably use an organic solvent complex including one 30 or more organic oil solvents together with a mutually oil and solvent-soluble substance which is capable of reacting with an alkaline compound to form an emulsifying agent. The solvent complex preferably includes a fatty acid, as the 35 mutually oil and solvent-soluble substance, the ingredients being preferably so chosen that the specific gravity of the mixture is substantially that of water.

By the use of this conditioning composition in 40 relatively small amounts mixed with, but not emulsified in a large amount of water, the oil and grease attached to the metal parts is brought into a state of mobility. In the second stage, there is used an alkaline compound which can 45 combine with the fatty acid or other mutually oil and solvent-soluble substance used in the first stage to form an emulsifying agent therewith.

The conditioning composition which is applied in the first stage is simply introduced into the 50 water-filled radiator, and the engine is allowed to run, thereby to cause the composition to circulate with the water for a period of time. Thereupon, the second stage of the operation is performed by adding to the circulating liquor of the 55

- first stage, a solution of an alkaline compound or an alkaline compound itself, in an amount in excess of that required to combine with the emulsifiable material added in the first stage, the mass being kept in circulation at an elevated temperature until all of the oil and grease has been loosened from the metal parts. The liquor is then drained out and the system flushed with water until thoroughly cleaned.
- 10 By the use of a small amount of organic solvent or solvent complex, coarsely dispersed but not emulsified, in a large amount of water, the bond between the emulsified grease and the metal surface is weakened. By coarse dispersion we means dispersion such that a large proportion of the oil will separate out in a relatively short time from the quiescent mixture. The addition to the mixture of an oil soluble material capable of reacting with alkali increases the emulsification of the grease which takes place during the second stage, for emulsification is apparently effected thereby throughout the entire mass so as to produce a state in which the grease particles seem entirely to lose their power of adherence. Thus, there is rapidly and inexpensively obtained, a degree of cleansing superior to that accomplished where either organic solvents alone or emulsions of such solvents in alkaline or saponaceous liquors are used.
- 30 The conditioning composition for the first stage, preferably includes a mixture comprising a hydrocarbon solvent of specific gravity less than water, a halogenated hydrocarbon solvent of specific gravity greater than water, and a fatty acid or vegetable oil or animal soap stock soluble in such hydrocarbon and halogenated hydrocarbon and more or less miscible with the oil or grease present, the relative proportions of such ingredients being preferably so determined that the specific gravity of the final mixture is substantially equal to that of water.
- Specifically, we may employ 1400 parts by volume of kerosene, 2275 parts of ortho-dichlorbenzol and 350 parts of oleic acid or red oil. This mixture is a substantially anhydrous liquid of the fluidity of a light oil.
- 50 In the example cited, the kerosene may be replaced by any other hydrocarbon solvent, as benzene or toluene, or any other water immiscible oil solvent such as a higher alcohol. In general, we prefer to use a solvent which does not boil at low temperatures and thus admits of use in hot radiator liquors. The ortho-dichlorbenzol may be replaced in whole or in part by any other halogenated hydrocarbon, as carbon tetrachloride, or even a non-halogenated oil solvent of proper specific gravity, but we prefer to use a halogenated compound because of the lessening of the fire risk inherent in the use of such compounds. For the red oil of the example cited above, we may substitute any other cheap fatty acid which may be available or any cheap saponifiable vegetable oil, such as cotton seed, coconuts or castor oil or an animal soap stock comprising a fat or oil, such as stearine.
- 60 The reaction composition applied in the second stage comprises any alkaline compound which is capable of reacting with the fatty acid or animal or vegetable oil or fat used in the mixture of the first stage to form a soap or an emulsion therewith. Specifically, sodium metasilicate may be used for this purpose, either in solid form or in solution, as it affords a particularly stable emulsion. The meta-silicate of soda may, however, be replaced by any of a wide range of other

alkaline compounds, such as caustic soda, tri-sodium phosphate, organic amines, hydroxylated amines or the like.

It is preferred to market our cleansing compositions in a composite wrapper including a package of the conditioning composition for the first stage, and a package of the reaction compound for the second stage. Ordinarily, there will be approximately four parts by weight of the first or conditioning composition to one part by 10 weight of the second or reacting compound. For a sixteen quart radiator, eight ounces of the preferred conditioning composition would, accordingly, be used to two ounces of the second or reaction compound. Preferably, after introduction of the conditioning composition for the first stage into the circulating system, the water is allowed to circulate by the operation of the water pump for about thirty minutes, at such temperature as the solution will acquire. Thereupon, the second or reaction compound is added and the circulation is maintained for about another ten to twenty minutes. The cleansing liquor may thereupon be drained, and the radiator flushed with water until all loosened dirt, 25 rust and grease have been washed out.

In the operation set forth, the first or conditioning composition being homogeneously distributed in the water within the radiator, since its specific gravity is that of water, effectively enters 30 into intimate engagement with the accumulation on the metal parts, especially as the grease solvent thereof has substantial wetting powers. The conditioning composition thus thoroughly soaks into the grease accumulation, fluffs it up somewhat and tends to loosen it. The alkaline or reaction compound added after this conditioning of the accumulation has occurred, promptly reacts with the red oil or equivalent ingredients of the conditioning composition and may also react with 35 some or all of the grease and oil to be removed from the wall, to form therewith either an emulsion or a soap. The emulsifying or saponifying reaction between the two batches of cleanser, occurs effectively in situ at the metal parts, so that 40 the accumulation becomes chemically and/or mechanically combined with the cleansing compound as the ingredients thereof react with each other, and thus the accumulation is entrained with the liquor. The excess of the alkaline compound of the second or reaction stage, not only assures an effective and complete reaction but also serves to soften the water, thereby to avoid any scale formation.

Although we have illustrated and described our 55 improved process, in its application to the removal of dirt, rust and grease from automobile radiator cores, we do not wish to limit ourselves to such application as our invention may be used to advantage, for the cleansing of other metal 60 parts by chemical means.

It will thus be seen that there is herein described a composition and method in which the several features of this invention are embodied, and which composition and method in their action attain the various objects of the invention and are well suited to meet the requirements of practical use.

As many changes could be made in the above composition and method, and many apparently 70 widely different embodiments of this invention could be made without departing from the scope thereof, it is intended that all matter contained in the above description shall be interpreted as illustrative and not in a limiting sense.

Having thus described our invention, what we claim as new and desire to secure by Letters Patent is:—

1. The method of cleansing metal parts fouled by oleaginous accumulation thereon, which consists in passing thereover a current of water and a mixture including a hydrocarbon solvent of specific gravity less than that of water, a halogenated hydrocarbon solvent of specific gravity greater than that of water and an oleaginous soap stock soluble in such hydrocarbons and miscible with the oleaginous ingredients to be removed, said mixture forming a coarse dispersion in water and being per se neither soluble nor emulsifiable therewith and after said composition has acted, adding to the liquor a water soluble alkali capable of combining with the said soap stock as well as the accumulation to be removed in one of the operations designated by emulsification and saponification. 5
2. The method recited in claim 1 in which the ingredients of the mixture, other than the alkaline material, are in proportion such as to have substantially the specific gravity of water. 10
3. The method of cleansing metal parts fouled by oleaginous accumulation thereon, which consists in passing thereover a current of water and a mixture including a hydrocarbon solvent of specific gravity less than that of water, a halogenated hydrocarbon solvent of specific gravity greater than that of water and oleaginous soap stock soluble in said hydrocarbons and miscible with the oleaginous ingredients to be removed, said mixture forming a coarse dispersion in water and being per se neither soluble nor emulsifiable therewith and after said composition has acted, passing over the metal parts the said current of water with water soluble alkali added thereto. 15
4. The method of cleansing the water circulating system of an internal combustion engine, which consists in adding to the circulating water a mixture including a grease solvent and a saponifiable oil, which mixture per se is neither soluble in nor emulsifiable with water permitting the liquor to circulate for a period of time and then adding thereto a water soluble alkaline substance capable of saponifying certain of the oleaginous constituents as well as certain of the oleaginous constituents of the accumulation to be removed from the walls of the system. 20
5. The method of cleasing the walls of the water circulating system of an internal combustion engine, which consists in adding to the water, a mixture of substantially the specific gravity of water, including a grease solvent of the group consisting of kerosene, benzene, and toluene, and an emulsifying agent of the group consisting of fatty acid, vegetable and animal fats and oils, which mixture per se is neither soluble in nor emulsifiable with water and after the circulation has proceeded for a period of time adding to the liquor, an alkali of the group consisting of sodium meta-silicate, tri-sodium phosphate and caustic soda and continuing the circulation of the liquor for a period of time. 25
6. The method of removing accumulation of grease, oil, rust and dirt from the water circulating system of an internal combustion engine, which method consists in adding to the circulating water, a conditioning composition comprising 1400 parts by volume of kerosene, 2275 parts of ortho-dichlorbenzol, and 350 parts of oleic acid said composition per se being neither soluble in nor emulsifiable with water permitting the water to circulate for a period in the neighborhood of 30 minutes at such temperature as it will acquire and then adding a water soluble alkaline reaction compound capable of saponifying oleic acid and continuing the circulation for a period in the neighborhood of 10 to 20 minutes. 30
7. The method of cleansing metal parts fouled by deposit thereon of oleaginous accumulation which consists in circulating water over the said metal parts having a conditioning composition distributed therein, the said composition and the ingredients thereof, being per se neither soluble in nor emulsifiable therewith and comprising mutually oil and solvent soluble soap stock and an organic oil and grease solvent, said composition forming a coarse dispersion in said carrier, and then applying a water soluble alkali and maintaining the carrier and the emulsion thus formed therewith in active movement in contact with the said metal parts. 35
8. The method of cleansing metal parts fouled by deposit thereon of oleaginous accumulation which consists in circulating water over the said metal parts having a conditioning composition distributed therein, the said composition and the ingredients thereof being per se neither soluble in nor emulsifiable therewith and including organic oil and grease solvent soluble soap stock, said composition forming a coarse dispersion in water, and then applying a water soluble alkali capable of promoting emulsification of an ingredient of said conditioning composition as well as an ingredient of the accumulation to be removed and maintaining the carrier and the emulsion thus formed in active movement in contact with the said metal parts. 40
9. A composition useful in one step of cleansing metal parts that have become fouled with oleaginous accumulation, said composition comprising a hydrocarbon solvent, of specific gravity less than one, a halogenated hydrocarbon solvent of specific gravity greater than one, and an ingredient of the group consisting of fatty acids, vegetable and animal soap stock, soluble in said hydrocarbon, said ingredients being in proportion such that the mixture has substantially the specific gravity of water said composition being of character which per se is neither soluble in nor emulsifiable with water. 45
10. A composition useful in one step of cleansing metal parts that have become fouled with oleaginous accumulation, said composition comprising a mixture of kerosene, ortho-dichlorbenzol and red oil and characterized by forming a coarse dispersion in water without solution or emulsification thereof the ingredients of said composition being in proportion such that the mixture has substantially the specific gravity of water. 50
11. A composition useful in one step of cleansing metal parts that have become fouled with oleaginous accumulation, said composition comprising a mixture by volume 1400 parts of kerosene, 2275 parts of ortho-dichlorbenzol and 350 parts of oleic acid and characterized by forming a coarse dispersion in water without solution or emulsification thereof whereby said composition in an aqueous carrier takes the form of a coarse dispersion which, when passed over the metal parts, softens the oleaginous accumulation so that the subsequent addition of water soluble alkali effectively emulsifies and removes the accumulation. 55